

Oct. 13, 1942.

E. REACH

2,298,724

METHOD OF MAKING ORNAMENTAL ARTICLES

Filed June 15, 1940

FIG. 1



FIG. 2



FIG. 3

Inventor

ERWIN REACH  
Edwin Reach

By

Attorney

## UNITED STATES PATENT OFFICE

2,298,724

## METHOD OF MAKING ORNAMENTAL ARTICLES

Erwin Reach, Hoboken, N. J., assignor to Jacob Firstenberg, doing business as Universal Importing Co., New York, N. Y.

Application June 15, 1940, Serial No. 340,644

3 Claims. (Cl. 18—61)

This invention relates to a method of producing ornamental articles.

One object of the invention is the provision of a method of producing from a plaster of Paris composition an article with a surface which is smooth and hard and capable of being polished to improve the appearance thereof and which is provided with an ornamental member of paper or the like.

A further object of the invention is the provision of a method of making a plaque or other article from a composition including plaster of Paris and other ingredients whereby the article has a smooth hard surface which is ornamented by attaching to the article during the molding or casting thereof a picture or other ornamental element of paper or other sheet material.

Another object of the invention is to provide an improved method of attaching the paper elements to the plaster plaques.

The above objects of the invention and other objects which might hereinafter appear will be fully understood from the following description considered with reference to the accompanying drawing.

In the drawing:

Fig. 1 is a sectional view of a mold and of a plaque formed therein in accordance with the present invention;

Fig. 2 is a front view of a plaque produced in accordance with the method illustrated in Fig. 1;

Fig. 3 is a sectional view on the line 3—3 of Fig. 2.

For producing the plaque or other article in accordance with the present invention there is utilized a mold 10 formed preferably of stainless steel or other material inert to the action of the plaster of Paris or other ingredients of the composition or other substances utilized in producing the article in said mold. The inner surface of said mold is preferably highly polished to provide the same with a very smooth and mirror-like finish. It will be understood that after each use of the mold for producing an article therein said surface is repolished whereby to renew said smooth and mirror-like finish thereof. A thin coating or film 12 of beeswax or similar material is applied to the polished surface of the mold, said coating of beeswax on said highly polished surface of the mold contributing to the provision of a smooth finish on the surface of the plaque or other article produced in said mold.

As illustrated in Fig. 2 the plaque 14 is provided with an ornamental insert 16, for example, paper or other suitable sheet material having a

picture lithographed or printed thereon. In producing the article with said insert the latter is preliminarily treated before placing the same in the mold. In this preliminary treatment of the insert, which ordinarily consists of paper having a picture printed thereon, said insert is immersed in water heated to a temperature between 185° F. and 225° F. depending on the weight of the paper. By thus subjecting the paper insert to the action of the water the paper is conditioned for effectively adhering to the plaster of Paris composition, this treatment of the paper serving to open the pores of the paper whereby to allow the casting composition to penetrate between the fibres of the paper. After the treatment of said paper insert with hot water, said insert is removed from the water and allowed to cool to atmospheric temperature and while still wet said insert is coated with a water solution of gum tragacanth, said gum tragacanth solution having the consistency of cream. The insert is then placed in the mold or form 10 in the proper position therein with the ornamented side of the insert coated with said film of gum tragacanth solution in contact with the coating of beeswax. The coating 11 of gum tragacanth on the insert serves to hold the same in proper position in the mold and in perfectly flat condition therein and in contact throughout its area with the flat surface of the mold, thereby to prevent air or other fluid bubbles between the insert and the mold surface. After the article is finished, the gum tragacanth film dries and is invisible on the insert. Also as said film dries it becomes greatly reduced in thickness, whereby the outer surface of the insert is offset inwardly from the outer surface of the plaque.

After the picture is properly positioned in the mold or form as described above, a solution of alum in water is applied, preferably by spraying by means of an air brush, on the inner surface of the mold over the coating of beeswax, and over the back of the insert, as indicated at 18 in Fig. 1. The proportion of alum in water is about 2% by weight of alum to about 98% by weight of water. The purpose of applying this substance on the surface of the mold is to form on the outer surface of the plaque or article a dense, hard and smooth layer 20 of the plaster of Paris composition. Said surface is extremely hard and smooth and can be highly polished. Then, while the film of alum is still wet, and while the insert is still wet the body portion 22 of the plaque is formed by pouring the plaster of Paris composition into the mold over said

insert to an appropriate depth in accordance with the thickness of the plaque or other article produced in said mold.

Said plaster of Paris composition consists of plaster of Paris, Tabioco dextrin or similar dextrin and water, in the proportion of about eleven pounds of plaster of Paris, six pounds of Tabioco dextrin or similar dextrin and seven pounds of water. The dextrin reduces the porosity of the casting composition and contributes to the formation of the provision of a surface which is hard and capable of being highly polished. In preparing the composition the water is preferably heated to about 90° F. or to some other temperature, then the dextrin or similar material is added to the water and finally the plaster of Paris is sifted into the water until it is completely dissolved. It will be understood that the casting composition is poured into mold 10 immediately after it is formed. This casting composition also preferably includes coloring materials or agents, the latter are inert to the ingredients of said composition. Said coloring agent is mixed therein in such manner as to obtain the desired effects, i. e., either solid color or onyx effects depending upon whether the coloring agent is completely mixed and uniformly distributed throughout the plaster of Paris composition or only partially or non-uniformly mixed therein whereby to leave uneven shadings or colorings which appear on the surface of the completed plaque or other cast article and impart thereto the onyx or marble appearance. Said coloring agent is preferably water soluble or in a solution which is miscible or compatible with or soluble in water.

After the plaster of Paris composition is cast in the mold and hardens therein the edges of the plaque are trimmed and the latter is removed from the mold and placed in a drying oven which is heated to a temperature of about 165° F. The plaque is allowed to remain in the oven until it is semi-dry and then removed from said oven and exposed to air at room temperature to complete the drying or setting process. Thereafter, the surface plaque is polished preferably by subjecting the same to the action of a polishing substance and a buffing wheel. The outer surface layer 20 of the plaque being extremely hard, smooth and of greatly reduced porosity, by reason of the composition of the casting material and the action thereon of the alum solution in the mold, that said surface can be and is highly polished so that the plaque has a hard, smooth and lustrous or glossy surface similar to that of onyx or marble. The polishing substance is preferably of the kind used for polishing stainless steel or other hard metals. Said buffing wheel preferably consists of a plurality of circular layers of buffing or polishing material separated from each other by cardboard disks which are smaller in diameter than the layers of buffing material whereby to provide spaces between the layers of buffing material for the circulation of air. A similar buffing tool is preferably utilized in applying the beeswax or similar material to the surface of the mold as described above.

After the polishing operation the plaque or other article 14 can have other operations performed thereon and other elements added thereto. For example, as illustrated in Figs. 2 and 3 a recess 24 is provided in the body portion of the plaque by removing a portion thereof in any suitable way as by drilling or milling the same from the body portion of the plaque to the desired depth, and any article, for example, a thermometer 26 carried by a mounting or backing plate 28, can then be inserted in said recess 24 and secured in position in any suitable way, for example, by a close fit in said recess and by an adhesive. Also, if desired, another article, for example, a calendar 30, can be attached to the outer surface of the plaque. Also, as here shown, said plaque can be provided with a hanger 32 which can be fastened to the plaque by inserting a hanger-forming element 32 in the composition in the mold as illustrated in Fig. 1 so that when the plaster of Paris sets said hanger-forming member is firmly attached to the plaque. Said member 32 can be formed of bendable sheet material so that the part projecting from the body portion of the plaque can be bent upwardly as illustrated in Fig. 3.

Thus, it is seen that the objects of the invention can be readily accomplished as described above. It will be understood, however, that the invention may be practiced otherwise than as hereinbefore specifically illustrated or described. Accordingly, I do not wish to be limited to the invention as herein shown or described except to the extent which may be required by the scope of the appended claims.

Having thus described my invention, what I claim and desire to secure by Letters Patent is:

1. The method of making an ornamental article in a mold, which comprises wetting a paper ornamental member, applying a coating of gum tragacanth to the outer or ornamental surface of said paper member, positioning said paper member while wet in said mold, and disposing a layer of plaster of Paris casting material in said mold over said paper member.
2. The method of making an ornamental article in a mold, which comprises wetting a paper ornamental member, applying a coating of gum tragacanth to the outer or ornamental surface of said paper member, positioning said paper member while wet in said mold, coating the inner surface of the mold with a solution of alum and disposing a layer of a plaster of Paris casting material in said mold over said paper member.
3. The method of making an ornamental article in a mold, which comprises coating the inner surface of said mold with beeswax, applying over said coating of beeswax a coating of alum, wetting a paper ornamental member, applying a coating of gum tragacanth to the outer or ornamental surface of said paper member, positioning said paper member while wet in said mold, and disposing a layer of plaster of Paris casting material in said mold over said paper member.

ERWIN REACH.